

3,415,051  
**PIECE-DYEABLE CARPET AND  
YARNS THEREFOR**

Raymond Adrian Levesque, Stamford, and Richard Cecil Newton, Norwalk, Conn., assignors to American Cyanamid Company, Stamford, Conn., a corporation of Maine  
No Drawing. Filed Apr. 13, 1966, Ser. No. 542,223  
8 Claims. (Cl. 57—140)

**ABSTRACT OF THE DISCLOSURE**

Piece-dyeable carpets of acrylonitrile polymer fibers and yarns for making such carpets are provided wherein such yarns are composed of bicomponent fibers of acrylonitrile polymer, the components of which have a shrinkage differential of 5-20% and substantially the same hydrophilic properties, the yarn developing in water at 200° C. a compression bulk of at least 6.0 cc./g. under a load of 18 g./inch of yarn and/or a specific bulk of at least 7.0 cc./g.

This invention relates to a method of making piece-dyeable carpet fabrics from yarns prepared from bicomponent fibers of acrylonitrile polymers. It relates further to the process of dyeing such carpet fabrics whereby the carpet fabric develops high bulk under hot-wet dyeing conditions and retains its bulk after being removed from the dyebath and dried. It relates further to the new carpet fabrics having the foregoing properties. Still further, it relates to the yarns used to prepare the said new carpet fabrics.

It is a well-known fact that bulky carpet fabrics provide covering power and a luxurious feel not found with carpet fabrics of the same material and weight, but with less bulk. The desirable property of bulkiness results from crimping in the fiber that makes up the carpet yarn. Crimped fibers cannot lay together as closely as the same fibers without crimp, and thus they stand apart from each other with the result that they occupy a relatively large amount of space. Acrylic yarns have been designed to have high bulk, and they have been used in carpet fabrics. However, there has been no satisfactory way to dye the fibers once they have been woven into a carpet since during the hot-wet dyeing operation conventionally used fibers tend to lose their crimp (i.e., they tend to "lean out"); the yarns consequently tend to lose bulk. Also, the carpet tufts tend to lean over and mat down (i.e., they tend to develop a condition known as "pile lay"). Furthermore, through loss of crimp or by failure to develop crimp, the weakly-held fibers are easily pulled out under the tension and abrasive action encountered by the carpet when it is dipped in and out of the dyebath, resulting in a fuzzy carpet surface. While the fuzz can be sheared from a carpet having a single level pile or the top level of a multi-level pile, it cannot be sheared from the lower levels of a multilevel pile. All these phenomena result in a "loss of value." These effects can be minimized, but only by costly special carpet constructions or elaborate post-dyeing procedures, e.g., jet steaming, back-beating, shearing, etc. In practice, all dyeing has been done either on the fiber itself (i.e. "stock" dyeing) or on the unwoven yarn ("skein" dyeing).

Both skein and stock dyeing involve some difficulties which would be desirably avoided, but unfortunately cannot be. In both processes an inventory of dyed fiber or yarn must be maintained for each carpet color in the manufacturer's line.

In view of these difficulties in the manufacture of acrylic carpet fabrics, it is an object of this invention to provide a commercially feasible method for the production of a

piece-dyeable carpet which does not require special carpet construction or expensive post-dyeing procedures for pile restoration, development of bulk and elimination of fuzz. An additional object is to produce a carpet which does not lose value during the piece-dyeing step. Still another object is to produce a piece-dyed carpet with reduced fuzz. A still further object is to produce a piece-dyeable, multi-level pile carpet. Still another object is to produce a piece-dyed carpet with improved firmness and little lean out or pile lay and high bulk and covering power. Yet another object is to provide a yarn suitable for the production of such carpets. Other objects will be apparent from the ensuing description of this invention.

In accordance with the present invention, these objects are achieved by providing a carpet fabric tufted of low twisted yarn composed of bicomponent fibers of acrylonitrile polymer whose monocomponent parts have substantially the same swelling potential, shrink 5-20% differentially, and develop under the conditions of hot-wet dyeing in a high degree of essentially irreversible and dimensionally stable crimp. Little or no further crimp is developed upon drying and the crimp is substantially permanent to subsequent hot-wet treatments. This characteristic is for convenience referred to as "irreversible crimp." Due to the self-crimping nature of these fibers, yarns comprised of such fibers develop a high degree of bulk which generally results in a yarn contraction of 10 to 40% during the dyeing step.

It is essential to the invention that all components of the composite fiber possess nearly comparable hydrophilic properties, i.e., the components must possess nearly comparable longitudinal and low radical swellabilities.

Fibers of the "irreversible crimp" type should not be confused with fibers of the "reversible crimp" type. Illustrative of reversible crimp fibers are those disclosed and claimed in U.S. Patent No. 3,038,236 and the rayon fibers in U.S. Patent No. 2,439,815. Illustrative of irreversible crimp fibers are those disclosed generally in U.S. Patents Nos. 2,439,815 (column 2 line 41 et seq.) and 3,182,106 as well as sample (B) of Example VI of U.S. Patent No. 3,038,236. It is noted above and has been found that such reversible crimp fibers cannot provide the advantages of the present invention since they develop most of their crimp only upon drying. Thus, in piece-dyeing carpets, fibers having reversible crimp will not crimp to a high degree when hot and wet; and the carpet is consequently beset with problems of pile lay, lean out and fuzz. The yarns of the present invention must develop during the dyeing step or other hot-wet processing to which the carpet fabric is exposed a specific bulk of at least 7.0 cc./g. and/or a compression of at least 6.0 cc./g.

By the term specific bulk is meant the volume to weight ratio of a dry yarn as determined by the following test at room temperature, hereinafter referred to as Test (A):

**BULK TEST A**

A 100 cm. length of yarn is weighed and its diameter measured with a vertically counted Federal® C81S thickness gauge. Ten thickness readings along the length of a yarn sample are taken by raising the pressure foot  $\frac{1}{8}$  inch above the yarn surface and allowing it to drop onto the yarn. The specific bulk is then calculated by the following equation:

$$\text{Specific bulk in cm.}^3/\text{g.} = \frac{\pi D^2 L}{4M}$$

D=yarn diameter in cm.

M=weight of yarn in grams

L=length of yarn in cm.

While the specific Bulk Test A above is a useful measurement of yarn bulk under constant load, the following compression bulk test (Test B) can be used to measure

bulk with increasing compressional loads. Such data can be used to determine the resistance of yarn bulk to tensile, compressive, and abrasive forces, said resistance being of particular importance to bulk stability.

By the term "compression bulk" is meant the volume to weight ratio of a wet or dry yarn as determined by the following test at room temperature, hereinafter referred to as "Test B".

#### BULK TEST B

A yarn sample is placed between two circular plates 10 each having a diameter of 1 inch. One plate is connected to a micrometer which measures the distance between the plates while the other plate is connected to a load cell which measures the force on the sample between the plates. A simultaneous record of plate separation and associated forces can, therefore, be displayed on an X-Y recorder. The bulk can be calculated at different loads from the plate separation by the following:

$$\text{Compression bulk} = \frac{\pi d^2 \times 10^6}{4 \times (\text{tex})}$$

*d*=distance in cm. between plates

*tex*=weight of yarn in gms./1000 meters.

Yarn shrinkage is measured as the difference in length of a single end of yarn with a load of 0.001 g./denier prior to and following exposure to boiling water for 30 minutes. The water is cooled to 120° F., then the yarn is removed and air dried. The measurement may be expressed as:

Percent shrinkage=

$$\frac{\text{original length} - \text{resultant length} \times 100}{\text{original length}}$$

Fibers of acrylonitrile polymer which will develop "irreversible crimp" may be obtained by co-spinning, side by side, two or more polymers of acrylonitrile of nearly identical swelling potential but of different comonomer proportions, each polymer containing at least 70% acrylonitrile. The components of the bicomponent fiber useful for the practice of the present invention have a differential shrinkage of about 5% to about 20%, and preferably of about 10% to about 15%. This means that one component will have a greater loss of original length upon shrinking than the other component by these amounts. This shrinkage differential induces a crimp in the composite filament. Too low a shrinkage differential results in a yarn which does not develop enough compression bulk to piece-dye satisfactorily. Too high a shrinkage differential results in a yarn which has a harsh hand. Also, a high shrinkage differential gives a high yarn shrinkage which, if too high, cannot be accommodated with existing carpet tufting equipment.

By "polymer of acrylonitrile" is meant a polymer composition which contains an average of at least about 70% acrylonitrile in the polymer molecules. When acrylonitrile is not homopolymerized, the remainder of the polymer molecules may contain an average of up to about 30% of another ethylenically unsaturated material as is well known in the art. Illustrative of these other compounds which may be copolymerized with acrylonitrile to form polymers which can be used in the practice of the present invention are those which may be found, for example, in U.S. Patent 3,104,938, issued Sept. 24, 1963, and U.S. Patent 3,040,008, issued June 19, 1962, and in the various other United States patents mentioned therein.

The individual bicomponent fibers used in the piece-dyeable carpet fabric of this invention resemble helical springs when viewed under a microscope. The coils of this spring will be in one direction for several coils and then in the other direction for several coils. These reversals, seen throughout the fiber length, are caused by restraints when the fiber crimp is developed and are believed to provide a higher yarn bulk than in fiber with a symmetrical helical shape. It may be visualized that this configura-

tion will resist deformation in any lateral direction unlike a fiber having only co-planar crimp.

To practice the present invention, bicomponent fiber of the type defined above is stretched at a temperature required to temporarily remove the helical crimp and is cooled under tension. After the fiber is mechanically crimped to give it co-planar bale crimp, it is cut into staple and converted to carpet yarn. The yarn is of relatively low bulk at this stage since the fibers therein do not exhibit their latent helical crimp. The yarn is converted into carpet fabric and then dyed.

The aqueous dyebath containing conventional acrylic dye must be at a temperature between about 180° and 270° F. While in the dyebath, the bale crimp disappears. The latent helical crimp is developed and the yarn in the carpet fabric becomes bulky. Intrinsic crimping forces are only slightly nullified by the tension involved in transporting the carpet in and out of the dyebath. The wet dyed carpet fabric is then dried conventionally.

20 The dyed carpet fabric thus produced, even without elaborate post-dyeing treatment, will be observed to be high in value in that it is of high bulk as compared to conventional carpet fabric of the same weight. It will have very little surface fuzz, will be substantially free of pile 25 lay or lean out, and in multi-level carpets, it will be free of fuzz on the lower levels as well.

It will be recognized, therefore, that great benefits are realized through the use of yarns of irreversibly self-crimping bicomponent fibers of acrylonitrile polymers, 30 which yarns develop bulk in hot water under tensions imposed by piece-dyeing, as described above.

While the present invention has been described and will be exemplified in terms of carpeting and yarn made of 100% irreversibly self-crimping bicomponent fibers, 35 it will be understood that it also includes the preparation of carpeting from yarns containing minor amounts of other fibers, e.g., monocomponent acrylic fibers, squirming bicomponent fibers, wool, nylon, etc. Likewise, while it is preferred to allow the hot-wet conditions incident to the dyeing operation to develop the bulk of the carpet yarn of the present invention, it will be understood that this invention also comprehends an operation whereby the carpet fabric is pre-bulked before dyeing. This pre-bulking operation can be accomplished by exposure to 40 either hot-wet or hot-dry conditions at any time prior to the dyeing operation. The carpet material with its pre-developed bulk may then be dyed by conventional means.

In the following examples presented to illustrate the present invention, some properties of carpet fabric are 45 determined by measurements on the yarns and fibers contained therein and other properties are determined by measurements on the carpets themselves.

#### Example 1

55 Two spinning solutions A and B were formed as follows:

| Component                                    | Solution A                         | Solution B                        |
|----------------------------------------------|------------------------------------|-----------------------------------|
| NaCNS                                        | 40 parts                           | 40 parts                          |
| Water                                        | 48.8 parts                         | 48.8 parts                        |
| Acrylonitrile/methyl-methacrylate copolymer. | 11.2 parts of 89.2/10.8 copolymer. | 11.2 parts of 91.7/8.3 copolymer. |

In a manner similar to that disclosed in commonly assigned copending application No. 249,203, filed Jan. 3, 65 1963, spinning solutions A and B were metered separately, but concurrently side by side through each hole of a spinnerette, at a weight ratio of 72 parts of solution A to 28 parts of solution B, into a sodium thiocyanate coagulating bath to form bicomponent filaments. The filaments were washed, stretched to 10 times their length and dried. These composite fibers were further subjected to steam under pressure at a temperature of 270° F. and allowed to shrink 40% of their stretched length. The resultant high degree of crimp was removed by restretching the fibers in a hot 1% aqueous solution of an anti-

static-lubricating textile aid, by the minimum amount sufficient to just remove said crimp. Minimum temperatures required to remove the crimp without damage to the fiber were used. The straightened fibers were mechanically crimped, dried and cut into 4 inch staple.

A sample of these staple fibers was exposed to water at the boil and dried. The dried fiber had a crimp frequency of 14.7 crimps per inch (c.p.i.) as compared to only 3.0 c.p.i. for the mechanically crimped fiber before exposure. Fiber shrinkage was 4.9% and fiber contraction (i.e., total change in length due to fiber shrinkage and crimp development) was 20.0%.

The mechanically crimped, undeveloped, staple fibers were processed into 2 ply 50's (Philadelphia count) greige carpet yarn of 4.0 t.p.i. (twists per inch) in singles and 2.5 t.p.i. in the plied yarn. The yarn had a specific bulk of 6.0 cm.<sup>3</sup>/g. After a sample of this yarn was immersed in boiling water and then dried, it had a specific bulk of 12.8 cm.<sup>3</sup>/g. and had shrunk 25.0%.

Multilevel pile carpet was made from the greige yarn and piece-dyed in equipment commercially used for piece-dyeing nylon carpet at 208° F. to 212° F. for 2½ hours followed directly by drying at 250° to 290° F. without jet-steaming, back-beating, shearing or any other special procedures. Examination of the dyed carpet before and after drying indicated that in both cases the tufts were erect and pattern definition was excellent. There was substantially no pile lay, no lean out, very little fuzz at any level and the carpet had a pleasant, firm hand which gave the impression of containing more fiber than a comparable weight stock-dyed acrylic carpet. There was no loss of value.

### Example 2

A bicomponent fiber was prepared as in Example 1 from 50 parts of solution A and 50 parts of Solution C of the following composition:

#### Solution C

|                                                  | Parts |
|--------------------------------------------------|-------|
| NaCNS                                            | 40    |
| Water                                            | 48.8  |
| Polymer of 94/6 acrylonitrile-methylmethacrylate | 11.2  |

A sample of the mechanically crimped fiber having 7.0 c.p.i. was immersed in boiling water and dried. After drying, it was found to have 15.5 c.p.i. Fiber shrinkage was 12.3% and fiber contraction was 41.2%.

The remainder of the fibers were processed into yarn as in Example 1. It had a specific bulk of 3.5 cm.<sup>3</sup>/g. A sample of the yarn was immersed in boiling water and then dried. It had a specific bulk of 8.5 cm.<sup>3</sup>/g. and had shrunk 30%.

The remainder of this yarn was tufted into carpet fabric and dyed as in Example 1. Examination of the dyed carpet fabric indicated substantially no pile lay, no lean out and very little fuzz at any level. Again, there was no loss of value.

### Example 3

Spinning solution A was extruded through a spinnerette into an aqueous sodium thiocyanate coagulating medium to form monocomponent filaments. The filaments were washed to further remove the solvent, stretched to ten times their extruded length, and then dried. The denier of the stretched fibers before drying was approximately 10 denier per filament. These fibers are identified as fiber 3A. Monocomponent fibers were spun under identical conditions from spinning solution B. These fibers are identified as fiber 3B. In a like manner, monocomponent fibers (identified as fiber 3C) were spun from a spinning solution C.

The dried fibers 3A, 3B and 3C, in a relaxed, unrestrained condition, were then steamed under pressure at temperatures in the range of 240° to 270° F. The amount of fiber shrinkage in each case at 10° increments over this temperature range is shown in Table I. Shrinkage was

calculated as the stretched length of the fibers minus the final relaxed fiber length divided by the final fiber length.

TABLE I

| Fiber | Shrinkage (Percent) |         |         |         |
|-------|---------------------|---------|---------|---------|
|       | 240° F.             | 250° F. | 260° F. | 270° F. |
| 3A    | 28                  | 31.5    | 36.0    | 44      |
| 3B    | 32                  | 32.5    | 33.0    | 34      |
| 3C    | 23.5                | 23.7    | 23.9    | 24.2    |

As seen from this table, shrinkage differentials of bi-component fibers can be controlled in the desired range of 5% to 20% by control of the steaming temperature of appropriately selected polymer compositions for each component.

Monocomponent fibers 3A, 3B and 3C were steam treated at 270° F., mechanically crimped and cut into 4 inch staple fiber. All fibers had essentially the same single filament properties with respect to crimp frequency and fiber shrinkage as shown in the following table:

TABLE II.—CRIMP FREQUENCY AND FIBER SHRINKAGE OF FIBERS 3A, 3B AND 3C

| Property        | Before boil-off<br>(measured dry) | After boil-off<br>(measured dry) |
|-----------------|-----------------------------------|----------------------------------|
| Crimp frequency | 8.0                               | 3.0                              |
| Fiber shrinkage | 2.0                               |                                  |

Each of the fibers was spun into 2-ply 50's resultant count carpet yarn of 4.0 x 2.5 twist. The resultant yarn count is the count (on the worsted system using Philadelphia counts) of the fiber after boiling, the yarn being originally spun to a lower count. Again, these yarns had approximately the same properties with respect to specific bulk and yarn shrinkage as shown in the following table.

TABLE III.—SPECIFIC BULK AND YARN SHRINKAGE OF FIBERS 3A, 3B AND 3C

| Property                      | Before boil-off<br>(measured dry) | After boil-off<br>(measured dry) |
|-------------------------------|-----------------------------------|----------------------------------|
| Specific bulk                 | 3.3                               | 4.0                              |
| Yarn shrinkage at .001 g./den |                                   | 6.0                              |

Yarn 3A was tufted into 32 oz./yd.<sup>2</sup> commercial multi-level (3/16", 5/16" and 7/16") carpets and piece-dyed in rope form in a dye beck at 200° to 210° F. An evaluation of the finished carpet showed severe lean-out, pile lay and considerable surface fuzz in the lower levels of the carpet.

In another test, when the carpets were subjected to the post-dyeing measures of jet steaming and back-beating to restore the pile and were then sheared to remove surface fuzz, the deficiencies noted above were somewhat diminished, but the carpet was still unsatisfactory and showed loss of value.

### Example 4

The following experiment was conducted to demonstrate the piece-dyeing technique as applied to a carpet prepared from producers high bulk yarn. Producers high bulk yarns are a blend of high-shrinkage and low shrinkage staple fibers.

Fiber 3A prepared from spinning solution A described in Example 3 was restretched 1.3 times its shrunken length in 180° F. water prior to crimping and staple cutting, thereby imparting a potential shrinkage of 23% upon re-exposure to 200° F. water. A staple blend of fibers containing 40% of the stretched fiber thus prepared and 60% of unstretched fiber 3A was made into 2-ply 50's resultant count carpet yarn as shown in Example 3. The resulting yarn had the following properties:

TABLE IV.—SPECIFIC BULK AND YARN CONTRACTION OF PRODUCERS HIGH BULK

| Property                                         | Before boil-off<br>(measured dry) | After boil-off<br>(measured dry) |
|--------------------------------------------------|-----------------------------------|----------------------------------|
| Specific bulk                                    | 3.0                               | 8.3                              |
| Percent yarn contraction at load of 0.001 g./den |                                   | 23.0                             |

It will be noted that the producers high bulk yarn developed a high degree of bulk after shrinking the untufted yarn in hot water.

The unbuked producers high bulk yarn of this example was tufted into carpets and dyed as in Example 3, employing post-dyeing corrective procedures designed to restore the tufts to an erect position and to eliminate fuzz. The carpet exhibited fair bulk and cover and very little lean-out. However, it had excessive fuzz on the lower level of the pile. The carpet had a loss of value and a mushy hand indicating a lack of firmness.

When the carpeting prepared above and dyed by the piece-dyeing method was not subjected to post-dyeing corrective procedures, the piece-dyed carpet was matted, due to pile lay. There was very little bulk or cover and the lean-out was excessive.

#### Example 5

This example demonstrates the difference in compression bulk values of various types of acrylic yarns: including yarns of this invention prepared as in Examples 1 and 2; yarns prepared from monocomponent acrylic fiber (the yarn of Example 3); producers high bulk yarns (the yarns of Example 4); and yarns prepared from Orlon® 33 acrylic fiber. The latter fiber is a blend of bicomponent fiber with reversible crimp and monocomponent fiber and has been reported in "Home Furnishings Daily" of June 17, 1965, to be useful in making commercially piece-dyeable carpets requiring post-dyeing restorative procedures. The bulk and shrinkage properties of the Orlon® 33 acrylic yarns are as follows:

TABLE V.—SPECIFIC BULK AND YARN SHRINKAGE OF ORLON® 33

| Property            | Before boil-off | After boil-off<br>(percent) |
|---------------------|-----------------|-----------------------------|
| Specific bulk.....  | 3.0             | 7.5                         |
| Yarn shrinkage..... |                 | 11                          |

The yarns of Examples 1 through 4 and Orlon® 33 acrylic yarn were exposed to a series of wetting and drying treatments which simulate piece-dyeing operations. These treatments are (1) exposure to 200° F. water for 5 minutes followed by (2) dipping in and out of 200° F. water (minimum time lapse) followed by (3) drying at temperatures up to 200° F. for 15 minutes. Tumble drying was used to simulate back-beating, a post-dyeing restorative procedure. The compression bulk of the yarn under increasing compressional forces was measured while the yarn was in the wet state and after it had been air dried or tumble dried. These values are given in the following table:

TABLE VI

| Fiber sample                         | Compression load, g./in. | Original<br>yarn bulk,<br>cc./g. | Static 5 min.<br>in 200° F.<br>water wet bulk | Dipping 5X in 200° F. water |                   |                              |
|--------------------------------------|--------------------------|----------------------------------|-----------------------------------------------|-----------------------------|-------------------|------------------------------|
|                                      |                          |                                  |                                               | Wet bulk                    | Air dried<br>bulk | 250° F. tumble<br>dried bulk |
| Example 1 (this invention).....      | 3.0                      | .....                            | 10.7                                          | 10.5                        | 15.7              |                              |
|                                      | 10.0                     | .....                            | 8.6                                           | 8.5                         | 11.0              |                              |
| Example 2 (this invention).....      | 3.0                      | 2.2                              | 8.4                                           | 7.5                         | 7.3               | 9.2                          |
|                                      | 10.0                     | .....                            | 10.6                                          | 10.5                        | 16.3              |                              |
| Example 3, Fiber 3A.....             | 3.0                      | .....                            | 9.0                                           | 9.1                         | 11.9              |                              |
|                                      | 10.0                     | .....                            | 7.7                                           | 8.0                         | 10.1              |                              |
| Example 4 (producers high bulk)..... | 3.0                      | .....                            | 8.5                                           | 8.0                         | 10.8              |                              |
|                                      | 10.0                     | .....                            | 6.2                                           | 5.8                         | 6.5               |                              |
| Orlon® 33 acrylic fiber.....         | 3.0                      | 3.0                              | 5.5                                           | 5.3                         | 4.9               | 5.3                          |
|                                      | 10.0                     | .....                            | 10.5                                          | 9.1                         | 18.5              |                              |
|                                      | 18.0                     | 1.8                              | 6.2                                           | 6.3                         | 6.3               | 9.2                          |
|                                      | 10.0                     | .....                            | 4.6                                           | 4.5                         | 5.2               |                              |
|                                      | 18.0                     | 3.0                              | 5.6                                           | 8.5                         | 12.1              | 19.0                         |
|                                      | 10.0                     | .....                            | 5.6                                           | 7.8                         | 13.4              |                              |
|                                      | 18.0                     | 3.0                              | 5.6                                           | 4.9                         | 5.8               | 10.3                         |

The foregoing data clearly show that the yarns of the present invention develop bulk in hot water and are able to retain the bulk despite the presence of increasing compressional forces both while the yarn is in the wet state and after it has been air dried. The yarns of the present invention are shown to be definitely superior in this re-

70 irreversible helical crimp, said yarn having a specific bulk of at least 7.0 cc./g. after exposure to water at 200° F.

7. Carpets prepared from the yarn of claim 5.
8. Carpets prepared from the yarn of claim 6.

gard as compared to the other yarns tested. This test, therefore, shows the superiority of the yarns of the present invention over the range of forces incurred during piece dyeing.

5 While the foregoing examples have illustrated embodiments of the present invention whereby bulk development has been accomplished under hot-wet conditions, it should be understood that the yarns of the present invention develop bulk under hot-dry conditions as well. Bulk developed this way is stable to subsequent hot-wet treatments and therefore is further resistant to loss by subsequent dyeing operations in the same manner and to the same extent as the yarns of Examples 1 and 2.

15 Moreover, though the foregoing examples have illustrated the improvement of the present invention whereby bulk development and dyeing were accomplished simultaneously in a dye bath, it should be understood that these two operations can be accomplished separately. Thus, the carpet of the yarn of the present invention may be subjected to hot-dry conditions or hot-wet conditions not connected with the dyeing operation to thereby produce an undyed carpet with developed bulk. The latter may then be dyed by conventional means.

We claim:

25 1. A yarn composed of bicomponent fibers of acrylonitrile polymer, the components of which have a shrinkage differential of 5-20% and substantially the same hydrophilic properties, the yarn developing in water at 200° F. a compression bulk of at least 6.0 cc./g. measured 30 under a load of 18 g./inch of yarn, said compression bulk being maintainable at a level of at least 6.0 cc./g. when subjected to the forces imposed by repeated dipping of the yarn in water at 200° F.

35 2. A yarn composed of bicomponent fibers of acrylonitrile polymer, the components of which have a shrinkage differential of 5-20% and substantially the same hydrophilic properties, the yarn developing in water at 200° F. a specific bulk of at least 7.0 cc./g.

40 3. A piece-dyeable carpet fabric prepared from the yarn of claim 1.

4. A piece-dyeable carpet fabric prepared from the yarn of claim 2.

5. Dyed yarn prepared from bicomponent fibers of acrylonitrile polymer, the fibers being characterized by 45 an irreversible helical crimp, said yarn having a compression bulk of at least 6.0 cc./g. measured under a load of 18 g./inch of yarn, said compression bulk remaining at a level of at least 6.0 cc./g. after being subjected to the forces imposed by repeated dipping in water at 200° F.

50 6. Dyed yarn prepared from bicomponent fibers of acrylonitrile polymer, the fibers being characterized by an

3,415,051

**9**

**References Cited**

**UNITED STATES PATENTS**

2,979,883 4/1961 Waltz ----- 57—140  
2,985,940 5/1961 Weldon ----- 57—140 XR  
3,081,516 3/1963 Evans ----- 57—140  
3,181,224 5/1965 Tanner ----- 57—140 XR

**10**

3,225,534 12/1965 Knospe ----- 57—140  
3,330,896 7/1967 Fujita et al. ----- 57—140

STANLEY N. GILREATH, *Primary Examiner.*  
5 W. H. SCHROEDER, *Assistant Examiner.*  
U.S. Cl. X.R.

28—72, 75